

May 15, 1928.

1,670,162

S. A. NEIDICH

COLLOID PRODUCT

Filed March 3, 1926

FIG. I.



FIG. II.



FIG. III.



FIG. IV.



FIG. V.



INVENTOR:

SAMUEL A. NEIDICH,  
By *Arthur E. Lange*,  
Attorney.

## UNITED STATES PATENT OFFICE.

SAMUEL A. NEIDICH, OF EDGEWATER PARK, NEW JERSEY.

## COLLOID PRODUCT.

Application filed March 3, 1926. Serial No. 91,961.

My invention is applicable in the manufacture of filaments by projecting viscose (cellulose sulphocarbonate) through orifices into baths containing chemicals which coagulate the viscose as a semi-solid impure cellulose hydrate of sufficient strength to be manipulated in the subsequent operations of dyeing, drying and weaving or braiding the same. Ordinarily, filaments projected through circular orifices and thus treated are solid cylinders of substantially uniform diameter and smooth exterior when dried. However, the purpose and effect of this invention is to produce a solid substantially uniform cylindrical filament surrounded by a tubular sheath which is crinkled so that its exterior surface presents numerous facets for reflection of light so as to have a scintillating effect, which is particularly desirable in the formations of braids, cords, etc., used in the millinery trade.

As hereinabove described; my invention includes the extrusion of primarily solid filaments of viscose, through suitable spinnerets, into a coagulating or precipitating medium, of such character as to immediately coagulate the exterior portion thereof, to such depth as to form what may be termed a skin, with the effect that, as the coagulation and reversion of the viscose within such skin proceeds, such stresses are created that, ultimately, the core comprising the entire substantially cylindrical body of the filament, within such skin, at some stage in its dehydration shrinks in diameter to such an extent as to pull loose from the skin, leaving the latter as a tubular sheath covering such cylindrical core throughout the length of the latter. However, during the desiccation of the structure as a whole, said sheath shrivels so that its exterior surface becomes crinkled and affords numerous irregular facets for reflection of light as aforesaid.

My invention includes the various novel features of construction and arrangement hereinabove more definitely specified. I have found that the effect aforesaid is producible by certain relations of the factors of strength of the precipitating bath, the speed of traverse of the filament through the bath and time of exposure of the filament to the action of the bath.

Ordinarily, aqueous solutions containing

eight percent of sulphuric acid or five percent of hydrochloric acid are considered strong coagulating baths and are commonly used for production of what are termed artificial silk filaments. However, it may be observed in the example of my invention hereinafter set forth that the acid strength of the bath is more than double such ordinary baths.

With baths of that character, substantially all of the sulphur primarily chemically combined with the cellulose in viscose is released as free sulphur and is occluded in the mass of cellulose hydrate, forms a dull yellow white surface upon the filament and renders the latter weak and brittle. It is practically impossible to more than partially remove sulphur and its derivatives from such cellulose hydrate by any ordinary process. However, I have discovered that if any suitable coagulating bath is made to include  $\text{PO}_4$  ions; filaments of cellulose hydrate formed by coagulating filaments in such baths are practically self-cleansing because the sulphur derivatives are thereby rendered soluble in the bath and automatically eliminated from the filaments. Such ions may be added to or produced in such baths in any convenient form or manner. However, trisodium phosphate ( $\text{Na}_3\text{PO}_4$ ) is a cheap vehicle for such ions and may be used in aqueous solution.

Therefore, in a preferable exemplification of my invention, I form a viscose precipitating bath of water containing sixteen and one half percent of  $\text{H}_2\text{SO}_4$ , in association with one half of one percent of  $\text{PO}_4$  ions, measured as  $\text{PO}_4$ , and cause the filaments to traverse such bath submerged in a path therethrough three and one half feet long and at the rate of one hundred twenty feet per minute; so that the time of subjection of each portion of the filament to such bath is one and three quarter seconds.

Although the peculiar effect aforesaid may be observed with a filament of three hundred denier, it is markedly characteristic of filaments between six hundred and one thousand denier and I prefer to utilize the same in filaments of nine hundred denier.

In said drawings: Fig. I is a perspective view of a piece of a finished product embodying my invention.

Fig. II is a fragmentary longitudinal sec-

tional view of an extruded viscose filament before coagulation.

Fig. III is a sectional view similar to Fig. II but indicating the coagulation of the exterior of said filament to form the skin aforesaid.

Fig. IV is a sectional view, similar to Figs. II and III but showing the core of the filament shrunken to such an extent as to be separated from its skin.

Fig. V is a fragmentary sectional view of the structure indicated in Figs. II to IV inclusive but in the final desiccated state and showing the core filament in elevation and the skin sheath thereof in section.

Referring to Fig. I, the complete product of my invention is an artificial thread, which may be woven, braided, knitted or otherwise embodied in any suitable texture and which includes the substantially smoothly cylindrical solid core filament 1 with the outer continuous imperforate tubular sheath 2 encasing said core in substantially coaxial spaced relation therewith but having a shriveled crinkled exterior affording multitudinous facets 3 adapted to reflect light with a scintillating effect.

Figs. II to V inclusive indicate steps in the production of such an artificial textile thread as indicated in Fig. I; by the exemplification of my invention above described.

Fig. II shows the solid homogeneous filament 4 of viscose, which, as extruded through a circular orifice, is substantially cylindrical and of homogeneous structure throughout its mass. Fig. III indicates the practically instantaneous effect upon the filament of Fig. II incident to its submersion in the bath above contemplated; which effect is the coagulation of the exterior of the filament 4 to such depth as to form what may be termed a skin 5. As the coagulation and reversion of the viscose within such skin proceeds, such stresses are created that, ultimately, the core comprising the entire substantially cylindrical body of the filament 4, within such skin 5, at some stage in its dehydration shrinks in diameter to such an extent as to pull loose from the skin, as indicated in Fig. IV, leaving said skin 5 as a tubular sheath 2 covering such cylindrical core throughout the length of the latter. During the continued dessication of the structure as a whole, said sheath shrivels so that its exterior surface becomes crinkled as indicated at 2 in Figs. I and V, and affords innumerable facets 3 for reflection of light, so as to have the desired scintillating effect. At such final stage of its production, both the interior core 1 and exterior sheath 2 have, of course, shrunken to much smaller diameter than the viscose filament from which they are formed. In fact an extruded viscose filament may shrink to one half its original diameter. Incidentally, the

shriveling of the outer sheath during the final dessication of the product, brings it into contact with the core filament at intervals throughout its length, and at some such regions of contact, the core and sheath adhere although retaining their distinctiveness incident to their primary separation throughout their length.

It is most economical to produce such threads in the least possible time of use of the apparatus employed and, therefore, it is desirable to run the extruded filament 4 through the bath at high speed as in the example above set forth. However, the desired effect may be attained in a somewhat weaker bath by longer subjection of the filament thereto; provided that the coagulating action thereof is strong enough to produce the skin effect described.

Moreover, although I prefer to include  $\text{PO}_4$  ions in the bath to avoid the necessity for using other desulphurizing methods and means to cleanse the product; of course, threads of the double character above contemplated may be produced in baths which do not contain  $\text{PO}_4$  ions, and such threads be subsequently desulphurized by any of the ordinary methods and means, well known in the art.

Furthermore, although I prefer to form such threads from the thiocarbonate of cellulose, known as viscose, as above described; containing about twelve per cent of cellulose, in hydrated form; there are at least four other methods of producing artificial colloid filaments in which my invention may be employed to wit, first, in the manufacture of filaments from nitro-cellulose by what is known as the Chardonnet methods and means; second, in what is known as the cuprammonium process, whereby filaments are formed from a solution of cellulose in an ammoniacal copper oxide; third, in the formation of filaments from a solution of cellulose in zinc chloride; and fourth, in the formation of filaments from acetic anhydride. Each of said processes and the methods and means for effecting the same are well known to those skilled in the art and, therefore, my invention may be applied thereto, in each case, by using such increased strength of the coagulating or precipitating medium that the ordinary purpose and effect of gradually coagulating the extruded filament throughout its mass so as to leave the latter of uniform and unitary composition, which is characteristic of the ordinary processes, are defeated by the instantaneous production of a substantially hard and tough skin upon the extruded filament capable of resisting the shrinkage of the gelatinous mass which it incloses; so that the subsequent desiccation of the latter causes it to separate from such skin. However, as above noted, in the finished product

- the tubular sheath and the core filament within it may come into contact and cohere, at intervals throughout their length, as a consequence of the shriveling of said sheath, 5 which produces the crinkled effect characteristic of my product.
- Therefore, I do not desire to limit myself to the precise details of construction, arrangement or procedure herein set forth, as 10 it is obvious that various modifications may be made therein without departing from the essential features of my invention as defined in the appended claims.
- I claim:
- 15 1. An artificial textile thread including a substantially smoothly cylindrical solid core filament and an outer continuous imperforate tubular sheath, encasing said core, in substantially coaxial, spaced, relation therewith, but having a shriveled crinkled exterior affording multitudinous facets adapted to reflect light with a scintillating effect; both said core and sheath being dry; said core being alternately adherent to, and in 20 radially spaced relation with, said sheath at intervals throughout their length.
2. An artificial textile thread including a solid core filament and an outer continuous imperforate tubular sheath, encasing said core, in spaced relation therewith, and having a shriveled crinkled exterior affording multitudinous facets adapted to reflect light with a scintillating effect; both said core and sheath being dry; said core being alternately adherent to, and in radially spaced 25 relation with, said sheath at intervals throughout their length.
3. An artificial textile thread including a solid core filament and an outer continuous imperforate tubular sheath, encasing said core, and having a shriveled crinkled exterior affording multitudinous facets adapted to reflect light with a scintillating effect; both said core and sheath being dry; said core being alternately adherent to, and in radially spaced 30 relation with, said sheath at intervals throughout their length.
4. A colloid product including a substantially smoothly cylindrical solid core filament and an outer continuous imperforate tubular sheath, encasing said core in substantially coaxial spaced, relation therewith, but having a shriveled crinkled exterior affording multitudinous facets adapted to reflect light with a scintillating effect; both said core and sheath being dry; said core being alternately adherent to, and in radially spaced 35 relation with, said sheath at intervals throughout their length.
5. A colloid product including a solid core filament and an outer continuous imperforate tubular sheath, encasing said core, and having a shriveled crinkled exterior affording multitudinous facets adapted to reflect light with a scintillating effect; both said core and sheath being dry; said core being alternately adherent to, and in radially spaced relation with, said sheath at intervals throughout their length.
6. A colloid product including a solid core filament and an outer continuous imperforate tubular sheath, encasing said core, and having a shriveled crinkled exterior affording multitudinous facets adapted to reflect light with a scintillating effect; both said core and sheath being dry; said core being alternately adherent to, and in radially spaced relation with, said sheath at intervals throughout their length.
7. A viscose product including a substantially smoothly cylindrical solid core filament and an outer continuous imperforate tubular sheath, encasing said core in substantially coaxial, spaced, relation therewith, but having a shriveled crinkled exterior affording multitudinous facets adapted to reflect light with a scintillating effect; both said core and sheath being dry; said core being alternately adherent to, and in radially spaced relation with, said sheath at intervals throughout their length.
8. A viscose product including a solid core filament and an outer continuous imperforate tubular sheath, encasing said core, in spaced relation therewith, and having a shriveled crinkled exterior affording multitudinous facets adapted to reflect light with a scintillating effect; both said core and sheath being dry; said core being alternately adherent to, and in radially spaced relation with, said sheath at intervals throughout their length.
9. A viscose product including a solid core filament and an outer continuous imperforate tubular sheath, encasing said core, and having a shriveled crinkled exterior affording multitudinous facets adapted to reflect light with a scintillating effect; both said core and sheath being dry; said core being alternately adherent to, and in radially spaced relation with, said sheath at intervals throughout their length.
10. An extruded colloid product including a solid core filament and an outer continuous imperforate tubular sheath, encasing said core, and having a shriveled crinkled exterior affording multitudinous facets adapted to reflect light with a scintillating effect; both said core and sheath being dry; said core being alternately adherent to, and in radially spaced relation with, said sheath at intervals throughout their length.
11. An extruded viscose product including a solid core filament and an outer continuous imperforate tubular sheath, encasing said core, and having a shriveled crinkled exterior affording multitudinous facets adapted to reflect light with a scintillating effect; both said core and sheath being dry; said core being alternately adherent to, and in radially spaced relation with, said sheath at intervals throughout their length.

core being alternately adherent to, and in radially spaced relation with, said sheath at intervals throughout their length.

12. An extruded viscose product including a solid core filament and an outer continuous imperforate tubular sheath, encasing said core, and having a shriveled crinkled exterior affording multitudinous facets adapted to reflect light with a scintillating effect;

said core being in contact with said sheath at intervals throughout its length; said core being alternately adherent to, and in radially spaced relation with, said sheath at intervals throughout their length. 10

In testimony whereof, I have hereunto signed my name at Burlington, New Jersey, this twenty-seventh day of January, 1926.

SAMUEL A. NEIDICH.